

# UNITED STATES PATENT OFFICE.

EMMET F. HITCH, OF ALTON, ILLINOIS, ASSIGNOR TO EQUITABLE POWDER MANUFACTURING COMPANY, OF EAST ALTON, ILLINOIS, A CORPORATION OF NEW JERSEY.

## PROCESS OF NITRATION.

1,198,129.

Specification of Letters Patent. Patented Sept. 12, 1916.

No Drawing.

Application filed April 17, 1915. Serial No. 22,129.

To all whom it may concern:

Be it known that I, EMMET FRANCIS Hitch, a citizen of the United States, residing at Alton, in the county of Madison 5 and State of Illinois, have invented certain new and useful Improvements in Processes of Nitration, of which the following is a specification.

This invention relates to processes of 10 nitration; and it comprises a method of nitration particularly adapted to aromatic hydrocarbons containing one or more methyl groups and to their mixtures but also applicable to the nitration generally of organic 15 bodies, and particularly where it is desired to cause an entrance of two or more nitro groups at the same time, wherein such material in a fluid state is admixed with a powdered solid nitrate, which is best sodium 20 nitrate and the mixture is then treated with a slight excess above the theoretical quantity of sulfuric acid, the amount of nitrate so used corresponding (with slight excess) to the number of nitro groups it is desired 25 to introduce; all as more fully hereinafter set forth and as claimed.

In the explosive industry there is a demand for explosive materials which shall be of a high degree of nitration (that is, 30 containing as many chemically combined  $\text{NO}_2$  groups in the molecule as possible) and shall also be liquid or soft and fluent. They should be substantially non-volatile at ordinary temperatures. High nitration is desirable as increasing the explosive power; liquidity or softness in nitrated products is desirable for many purposes. For example in making gelatinized explosives (such as gun-cotton made into a gelatinous mass with 35 nitroglycerin) there is a demand for a non-volatile liquid material which is in itself explosive and which can be added to the mixture to restrain the tendency of nitroglycerin to freeze in cold weather. Material of this kind is also desirable as a direct addition to nitroglycerin intended for use in making dynamite. In making explosive mixtures with the usual oxidants or oxygen-bearing salts, nitrates, perchlorates, 45 permanganates, chlorates and the like, such a material is also desirable since it renders possible the production of plastic compositions not readily affected by moisture. A

chlorate, such as chlorate of potash or chlorate of soda, for instance, although 55 *per se* a valuable oxidant in making mixed explosives is of restricted use since it is not safe in dry compositions while with most oily materials too much oil must be used in order to utilize the oxygen of the chlorate; that is the quantity of oil necessary 60 is too great for a uniform, easily handled mass.

The best materials for the stated purposes are the nitro derivatives of the aromatic 65 hydrocarbons or the phenols; the nitro derivatives of benzol, toluol, (methyl-benzene), the xylols, naphthalene, anthracene, phenol, the cresols, etc., since they are stable 70 bodies of good explosive power; but unfortunately when nitrated to a high degree these materials mostly furnish solid bodies, or substances crystallizing readily at moderately low temperatures. The lower nitration products, such as the mononitro 75 compounds, are often, but not always, fluid; the dinitro compounds are mostly solids but nearly all the trinitro compounds are solid and have a relatively high melting point. The higher nitration products are also 80 somewhat expensive to make by the usual methods since their production usually requires a double nitration; as by nitrating first with nitric acid and subsequently with a mixture of nitric acid and sulfuric acid. 85 With toluene (toluol) the mononitro products are fluid and the dinitro and trinitro products are solids at ordinary temperatures when in a state of purity. To make materials from toluene containing any great 90 amount of trinitro compounds ordinarily requires a double nitration with intermediate treatments which add to the expense. Further, by the nitration methods in use an excess of nitric acid is always used and this 95 excess must subsequently be recovered.

There are now in commercial use certain liquid nitro toluenes with a percentage of nitrogen above that corresponding to dinitro toluene, which are known to the trade as 100 "liquid trinitro toluene". These compositions are made by dissolving greater or less amounts of commercial solid trinitro toluene in mixtures of mono- and di-nitro toluenes. Such mixtures however are not satisfactory 105 for the stated purposes. On long standing

at moderately low temperatures, the trinitro toluene components tend to separate out more or less entirely in granular form or to form with the liquid nitro oils a composition of a pasty consistency. This separation of the trinitro toluene is due to the fact that the solutions when prepared in this manner are supersaturated and also to the fact that some of the volatile mono-nitro toluenes which act as solvents escape by evaporation on long standing. This volatile nature of the so-called liquid nitro toluenes is especially objectionable when they are used in the manufacture of gelatinized or plastic explosives since the explosives so made have a tendency to "freeze" more and more readily on standing.

Upon the general principle that with any mixture of two substances the melting point is below the average of those of the two substances in a pure state, the melting point of a mixture of high nitrated aromatic hydrocarbons or phenols can be very much reduced by having the mixture comprise a sufficient number of chemically different nitro bodies. Of this principle I take advantage in the present invention.

As my raw material I advantageously use coal tar oils, either the light tar oils or the heavy tar oils; or both together. Phenolic bodies may or may not be removed. The coal tar oils are composed of a large number of different hydrocarbons of the aromatic series, of benzene, methylbenzene (toluene), dimethylbenzenes (the xylols), ethylbenzene, etc., all susceptible of yielding nitro products of good explosive qualities. But it has heretofore been found difficult with any of these hydrocarbons, or with the oils themselves, to produce in any simple way or by any simple operation high nitro derivatives; derivatives containing more than one nitro group. In the art where high nitrated derivatives are desired it is, as stated, customary to nitrate in two or more steps; a mononitro compound being, for example, first formed and this afterward converted into di and tri compounds. For example, toluene is first nitrated to form a mixture of the three mononitro derivatives and then these mono derivatives are afterward renitrated to give the di and tri compounds. I have discovered however that by the use of a special method of nitration it is possible to obtain directly these highly nitrated derivatives without the stagewise procedure of the prior art; such method being applicable either to the separate hydrocarbons, or, and advantageously for the present purposes, to mixtures of these hydrocarbons. In such method, in lieu of using the ordinary direct nitration with nitric acid or with a mixture of nitric and sulfuric acids I employ a special procedure. To this end, I mix the material in

liquid form with a powdered solid nitrate, which is best nitrate of soda, although nitrate of potash may be used. Calcium nitrate is not so advantageous. If the material is not a liquid it may still be used if it can be melted by a moderate degree of heat, say, below 90° centigrade. The powdered nitrate is best quite finely divided, being, say, of such a fineness as to pass a 60 mesh sieve. The proportions of the material and of nitrate will depend upon the particular degree of nitration desired in the ultimate product as hereinafter set forth; but in all cases the proportions of solid to liquid are such that the mixture will be of a more or less pasty consistency, with the fluid material uniformly distributed and filming the faces of the particles of solid nitrate. This uniform distribution of solid nitrate and liquid material is an important feature in the present process. To this mixture I add sulfuric acid slowly with careful regulation of the temperature and energetic mixing and stirring. Ordinarily the temperature during this operation should not rise much above 90° C. and it may be much lower. After the full quantity of acid has been added mixing may be continued for an hour, or thereabout. Finally stirring may be discontinued and the material heated to about, say, 100° C. for an hour or so and thereafter the heat increased to 120° or 150°, heating at the higher temperature being continued until oxids of nitrogen cease to be evolved.

In the method of operation just described the nitric acid liberated from the nitrate by the sulfuric acid is directly presented to the compound to be nitrated as fast as formed and in a condition of maximum strength and dryness. Nitration is rapid and complete. To all intents and purposes the material and the nitrate are presented simultaneously to the action of the sulfuric acid; this being a very important point. In any nitration where the sulfuric acid has an opportunity to act directly upon the material there is a tendency toward the formation of sulfonic compounds as in cases where the material is preliminarily dissolved in or mixed with the sulfuric acid, as is sometimes recommended. Some of these sulfonated bodies are converted into nitro compounds with some difficulty. But where nitrate of soda and an organic body, such as toluene, are simultaneously, so to speak, presented to the sulfuric acid the sulfuric acid combines with the soda of the nitrate and the nitric acid thereby freed combines with the organic material. It is found in the present invention that the nitric acid so developed in what may be called a nascent condition, gives a smoother and more rapid nitration and a more uniform and higher nitration product.

In the present method the utilization of the nitric acid of the nitrate in the formation of nitro compounds is nearly the theoretical amount, but a slight excess of 5 nitric acid over the theory being required. Further, I have found that I can control the degree of nitration by the amount of nitrate used; or, stated in another way, I can at pleasure directly produce mono, di or tri 10 nitro compounds by using the corresponding amounts of nitrate. In the production of nitro-toluenes, for example, with one proportion of nitrate of soda I make the mono nitro compound; with double the amount I 15 produce a mixture of the three dinitro bodies, and with triple the amount I can produce highly nitrated compositions containing the tri derivatives.

With the aid of the described method 20 using the complex mixtures or hydrocarbons found in coal tar oils, I can produce compositions which are highly nitrated and at the same time are permanently fluid and substantially non-volatile at ordinary 25 temperatures. This is for the reason that the process produces so many nitro products from the many hydrocarbons that their mutual influence in reducing the fusing point makes the final composition fluid at ordinary 30 temperatures.

I can also use the described process of nitration for many materials not usually presumed to be nitratable. I have succeeded in nitrating mineral oils, both those of par- 35 affinic nature and those of naphthenic or quasi-aromatic nature, as well as vegetable and animal oils and many other liquid or readily fusible solid substances; liquid or fusible enough to film over the nitrate frag- 40 ments at a temperature not too high for nitration; say about 90° or 100° C.

I have found that the nitratability of these other materials may be advanta- 45 geously utilized in the specific invention herein described and claimed in that I may add a modicum of such material as rosin, 50 rosin oil, lubricating oil, vaseline, kerosene or the like to the tar oils prior to nitrating.

Co-nitration of these mineral oil materials 55 with tar oils, etc., further increases the complexity of the final product and to that extent still further reduces the melting or freezing point.

In a specific embodiment of the present 60 invention I may take about 100 parts by weight of light tar oil, say the fraction dis- 65 tilling between 100° and 120°, thoroughly mix the oil in a dry condition with, say, 250 parts of dry nitrate of soda, ground to 60 mesh. Incorporation of liquid and solid should be as intimate as possible. To this mixture I then add 450 parts of sulfuric acid; the ordinary commercial strength of 1.84 specific gravity serving very well. The 65 use of fuming sulfuric acid, or of acid en-

riched with SO<sub>2</sub>, while it may be practised, does not give substantially better results. The addition of sulfuric acid is best rather slow and energetic stirring should be resort- 70 ed to in order to obtain with certainty the desired simultaneous contact of the sulfuric acid with the oil and with the nitrate. During this stage of the operation the tempera- 75 ture tends to rise and it should be regulated so that it shall not go much above 90° C. The precise temperature to be used however depends in a measure upon the particular materials treated and the end product de- 80 sired. With light tar oils in making freely fluid end products of high nitration, about 90° C. is a good temperature of operation. After all the acid is added, stirring may be continued for an hour in order to produce completeness of reaction. Then the mixture may be warmed until it reaches about 100° C., at which temperature it may also be kept for about an hour. Finally the temperature may be gradually increased to about 150° C., being kept at this temperature until oxides of nitrogen are no longer evolved. When this point is reached, the lower semi-liquid layer containing the excess of acids and sodium bisulfate may be separated from the upper layer of nitrated oils and the nitrated oils washed and purified in any of the usual 95 ways.

The mixture of nitro products formed as just described is an oily body of a high degree of nitration, containing about 15 to 16 per cent. of nitrogen, and retains its fluidity 100 even at low temperatures. It is an excellent "anti-freezing" addition to nitroglycerin and to the various nitroglycerin compositions such as blasting gelatin. Used with perchlorate, chlorate or nitrate of soda or 105 potash or mixtures thereof it will furnish the necessary carbon and hydrogen for the utilization of the oxidizing energy of these substances, forming plastic substances without giving an unhandy bulk of liquid. Nor 110 are its vapors or fumes poisonous or offensive in manufacture or use as is the case with some nitro-compounds.

In making a high nitrated liquid product 115 from toluene I may use 25 parts of nitrate of soda to 10 parts of ordinary commercial toluene and 45 parts of sulfuric acid, fol- 120 lowing the procedure above indicated. The final temperature should not be over 120°. The result will be the formation of a perma- 125 nently liquid composition rich in trinitro compounds and substantially free of mono-nitro compounds. If complete conversion into trinitro compounds is required, the operation of nitration may be repeated. In nitrating toluene to produce fluid products a first nitration temperature of around 90° is desirable.

Dinitro toluene mixtures containing the 130 three dinitro bodies in varying proportions

may be readily made under the described method by reducing the amount of nitrate just indicated to 19 parts per 10 parts of toluene. By performing the nitration at the 5 temperature above described, viz., around 90° C., the proportion of metadinitrotoluene may be raised as high as 30 per cent.

In nitrating mixtures of aromatic hydrocarbons, or of tar oils, with other hydrocarbons or oils, such as petroleum oils, in the present manner, apparently a far-going nitration of the petroleum oils may be attained when the percentage of petroleum oil is not above 15 per cent.; that is, the nitrogen percentage of the finished nitrated composition does not differ materially whether small amounts of petroleum oils are in the initial mixture or not. This fact enables the use of rather impure or low grade oils or distillates analogous in general character to the coal tar oils, such as those made in various processes of converting petroleum oils into benzol, toluol and the like, since the presence of residual non-aromatic or petroleum oils 5 in small amounts does not interfere with the process. Similarly many shale oils, brown coal tar oils, etc., may be used, alone or in admixture with coal tar oils. Naphthenic oils, such as are obtained from California, 10 Texas and Mexican oils may also be used in admixture with coal tar oils and in somewhat greater proportion than is the case with ordinary vaseline or with paraffinic oils.

I find that mixtures containing a small proportion of a petroleum oil or petroleum material, such as vaseline, lubricating oil, etc., are advantageous as they nitrate rather more readily and smoothly; this being possibly due to the petroleum oil acting, so to speak, as a carrier of nitro groups in nitration. The final products are also somewhat more fluid.

Petroleum products while they may be nitrated alone do not ordinarily give end compositions which are as good alone as those obtained from tar oils. However by repeating the operation, more nitro groups can be introduced and the explosive qualities raised.

For practical purposes I prefer to nitrate the methylated or ethylated hydrocarbons of the benzene series since the nitro products yielded are better explosives. And by using the mixture of these hydrocarbons found in tar oils I obtain still better products than by using the pure hydrocarbons.

I regard the stated method of nitration as one of a quite general applicability although particularly advantageous for tar oils and their contained hydrocarbons. It is particularly advantageous in nitration where it is desired to introduce more than one nitro group.

The described process may also advantageously be applied to the treatment of naphthalene or of mixtures of naphthalene with petroleum oils. Naphthalene with 5 or 10 per cent. of lubricating oils forms a fluid 70 composition well suited for nitrating in the manner described. But naphthalene alone may be melted and so treated. It is advantageous however in operating with naphthalene for the sake of greater fluidity of the 75 final products, to use some tar oil as well as some petroleum material. Anthracene and anthracene oil (dead oil) may also be used. Rosin and rosin oil may also be used. Like petroleum materials they are best used as 80 adjuncts to the aromatic oils, such as coal tar oils. Rosin may be used in slightly larger amounts than rosin oil.

The complex, highly nitrated compositions obtained by nitrating tar oils in the 85 described manner, with or without admixed petroleum materials are, as stated, because of their fluidity or their low melting or freezing point, and non-volatile nature particularly well adapted for use in making 90 mixed gelatinized and plastic explosives, such as nitroglycerin mixtures, mixtures with oxygen-bearing salts such as perchlorates, permanganates, chlorates, nitrates, picrates, etc.

The present process may also be applied to liquid and easily fusible phenolic materials, or mixtures of such materials with hydrocarbons; such as phenol (carbolic acid), the cresols, creosote oils from coal 100 tar, wood tar creosotes, etc.

What I claim is:—

1. The process of nitrating organic bodies for the production of compounds containing two or more nitro groups wherein such a body in a fluid state is admixed with a solid nitrate in amount sufficient to correspond to the number of nitro groups desired in the product and the mixture so formed is treated with sulfuric acid. 105

2. The process of making permanently liquid, non-volatile polynitro compounds of methylated aromatic hydrocarbons which comprises admixing such a hydrocarbon in a liquid state with a solid nitrate in amounts 110 sufficient for the production of a trinitro compound and thereafter treating the mixture with sulfuric acid.

3. The process of making nitro compounds of aromatic hydrocarbons which 115 comprises admixing such a hydrocarbon in a liquid state with a solid nitrate and thereafter treating the mixture with sulfuric acid.

4. In nitration the process which comprises mixing a liquid organic body with a powdered nitrate to produce an intimate mixture and adding sulfuric acid to the mixture so obtained. 125

5. The process of obtaining polynitro com- 130

5 pounds which comprises admixing an organic body in a liquid state with an amount of a solid nitrate more than corresponding to the mononitro derivative of such organic body and thereafter treating the mixture with sulfuric acid.

6. The process of obtaining nitrocompounds of aromatic hydrocarbons of lowered fusing point which comprises admixing a material comprising such aromatic hydrocarbons with a material comprising petroleum hydrocarbons, adding the mixture in liquid form to a solid nitrate and producing intimate incorporation and thereafter adding sulfuric acid to the mixture.

10 7. In the nitration of tar oils, the process which comprises admixing such oil with a solid nitrate and thereafter treating the mixture with sulfuric acid.

20 8. The process of obtaining nitrocompounds of aromatic hydrocarbons of lowered fusing point which comprises admixing a material comprising such aromatic hydrocarbons with a material comprising another nitratable organic material, adding the mixture in liquid form to a solid nitrate and producing intimate incorporation and

thereafter adding sulfuric acid to the mixture.

9. The process of nitration which comprises mixing a solid finely powdered nitrate with enough of liquid organic body to film coat the grains thereof and thereafter treating with sulfuric acid.

10. The process of nitration which comprises mixing a solid finely powdered nitrate with enough of liquid organic body to film coat the grains thereof and thereafter treating with sulfuric acid at a temperature maintained around 90° C. during the period of energetic action.

11. The process of nitration which comprises mixing a solid finely powdered nitrate with enough of liquid organic body to film coat the granules thereof, treating with sulfuric acid, restraining the temperature during the period of energetic action to a temperature around 90° C. and thereafter raising the temperature to expel nitrous fumes.

In testimony whereof, I affix my signature.

E. F. HITCH.